

## UNITED STATES PATENT OFFICE.

TRUMAN S. FULLER AND DAVID BASCH, OF SCHENECTADY, NEW YORK, ASSIGNEES  
TO GENERAL ELECTRIC COMPANY, A CORPORATION OF NEW YORK.

## ALUMINUM ALLOY.

No Drawing. Continuation of application filed December 13, 1923, Serial No. 680,516. This application filed December 13, 1924. Serial No. 756,822.

*To all whom it may concern:*

Be it known that we, TRUMAN S. FULLER and DAVID BASCH, citizens of the United States, residing at Schenectady, in the county of Schenectady, State of New York, have invented certain new and useful Improvements in Aluminum Alloys, of which the following is a specification.

The present invention is a continuation of our application, filed December 13, 1923, Serial No. 680,516, and comprises an improved alloy of aluminum, zinc and magnesium, which is of particular utility for the manufacture of castings.

Alloys comprising these ingredients have been known heretofore in which a content of magnesium of a few per cent has been accompanied by a zinc content of approximately 20% or conversely in which a magnesium content of as high as 10% has been accompanied by the low zinc content of about 1%; also alloys are known containing a fourth ingredient, such as iron, in addition to the three ingredients mentioned.

We have discovered that an alloy of exceptionally good physical properties results from the combination of aluminum, zinc and magnesium in the proportions of about 3 to 8 parts zinc and about 0.25 to 1.5 parts magnesium, the balance of the alloy being aluminum except, of course, for incidental impurities.

In our above prior application, Serial No. 680,516, we have described a cast alloy comprising about 92.75 parts aluminum, about 6 parts zinc and about 1.25 parts magnesium which has a tensile strength of about 26,000 pounds per square inch and a hardness of about 75 Brinnell. The elastic limit (proportional limit) of this alloy is about 12,000 pounds per square inch. Although for some purposes this alloy is entirely suitable without further treatment, its properties may be improved by heat treating. For example, the alloy is heated to about 515° C. for about twenty-four hours, then is quenched in boiling water and finally is aged either artificially at about 150° C. for three hours or

more, or naturally. By this treatment the tensile strength is increased to about 35,000 50 pounds per square inch and the hardness is raised to about 104 Brinnell.

A cast alloy containing 0.5 parts magnesium and 5 parts zinc, the balance being aluminum (except for impurities) has an 55 ultimate tensile strength of about 24,000 pounds per square inch. The elastic limit of the alloy is about 7,000 to 8,000 pounds per square inch. The "elongation" of the alloy as measured by the tensile strength 60 tests is about 4 to 8 per cent.

In general in an alloy constituting our invention, the proportion of zinc preferably is maintained within the limits of about 4 to 6 per cent, and the proportion of magnesium preferably is maintained within the limits of about 0.5 to 1.25 per cent. As already indicated, good results are obtained even when the zinc content is as low as three or as high as eight per cent or when the 70 magnesium content is as low as 0.25 or as high as 1.5 per cent.

An aluminum alloy having a composition within these limits flows freely in a mold, forms castings having sharp outlines and 75 may be readily worked by machine tools.

It may be used either without heat treatment in the state obtained by casting or when improved by heat treatment.

What we claim as new and desire to secure 80 by Letters Patent of the United States, is:

1. An alloy consisting essentially of aluminum, zinc and magnesium, the zinc content of said alloy being within the limits of about three to eight per cent and the magnesium content being within the limits of about 0.25 to 1.5 per cent.

2. An alloy suitable for casting essentially consisting of about 0.5 to 1.25 per cent of magnesium, about 4 to 6 per cent of zinc, the balance of the alloy being aluminum except for incidental impurities.

In witness whereof, we have hereunto set our hands this 17th day of December, 1924.

TRUMAN S. FULLER.  
DAVID BASCH.